# EUROPEAN PATENT SPECIFICATION

(11) **EP 1 871 947 B1**
(45) Date of publication and mention of the grant of the patent: **25.05.2016**
(21) Application number: 06725251.0
(22) Date of filing: 22.03.2006
(51) Int. Cl.: D06M 23/10, D06M 23/08, C09D 11/00, D06B 9/00, B41J 3/407, D06B 11/00

(54) **COMPOSITION FOR DROP ON DEMAND FINISHING OF A TEXTILE ARTICLE**
ZUSAMMENSETZUNG FÜR DROP-ON-DEMAND-AUSRÜSTUNG EINES TEXTILERZEUGNISSES
COMPOSITION POUR FINISSAGE PAR GOUTTELETTES A LA DEMANDE D'UN ARTICLE TEXTILE

(30) Priority: 22.03.2005 GB 0505894
(43) Date of publication of application: 02.01.2008
(73) Proprietor: Ten Cate Advanced Textiles B.V., 7443 PV Nijverdal (NL)
(72) Inventor: CRAAMER, Johannes A., NL-8651 EG IJlst (NL); FOX, James E., Royston Herts, SG8 0PT (GB)
(74) Representative: Nederlandsch Octrooibureau
(86) International application number: PCT/EP2006/060969
(87) International publication number: WO 2006/100277

(56) References cited:
- US-A- 5 310 778
- US-A1- 2002 192 366
- US-A1- 2003 081 094
- US-A1- 2003 176 534
- US-A1- 2004 052 957
- US-B1- 6 328 393

## Description

### BACKGROUND OF THE INVENTION

### 1. Field of the Invention

The present invention relates to finishing textiles and more particularly to finishing of textiles by digital droplet deposition using drop-on-demand inkjet (DoD) techniques. It relates furthermore to finishing compositions specially adapted to this purpose and methods of performing such finishing.

### 2. Description of the Related Art

The production of textiles traditionally takes place in a number of distinct processes: the fibre production; spinning of the fibres; the manufacture of cloth (for instance woven or knitted fabrics, tufted material or felt and non-woven materials); the upgrading of the cloth; and the production or manufacture of end products. Textile upgrading is a totality of operations which have the purpose of giving textile the appearance and physical characteristics that are desired by the user. Textile upgrading comprises of, among other things, preparing, bleaching, optically whitening, colouring (dyeing and/or printing)and finishing a textile article.

The conventional process for upgrading textile is built up (see figure 1) of a number of part-processes or upgrading steps, i.e. pre-treating the textile article (also referred to as the substrate), dyeing the substrate, coating the substrate, finishing the substrate and the posttreatment of the substrate.

A known technique for printing textile is the so-called template technique. Ink is applied to cut-out leaves or elements, the templates, with which desired patterns such as letters and symbols can be applied to the substrate. Another known technique for printing textile is the so-called flatbed press technique, wherein the printed image lies in one plane with the parts of the print mould not forming a printing area. An example hereof is a so-called offset print, wherein the printing process takes place indirectly. During the printing the print area is first transferred onto a rubber fabric tensioned round a cylinder and from there onto the material for printing. A further technique is screen-printing, wherein the substance for applying is applied through openings in the print template onto the textile for printing.

As is already indicated in figure 1, dyeing of the substrate is another upgrading step. Dyeing is the application of a coloured chemical substance in a full plane, and then uniformly in one colour. Dyeing takes place at present by immersing the textile article in a dye bath, whereby the textile is impregnated with a coloured substance, visible on both sides of the substrate.

One form of finishing is coating. Coating of a textile involves the application of a thin layer to the textile to endow it with particular functional properties such as to protect or increase the durability of the substrate. The usual techniques for applying a coating on solvent or water basis are the so-called "knife-over-roller", the "dip" and the "reverse roller" screen coaters. A solution, suspension or dispersion of a polymer substance in water is usually applied to the cloth and excess coating is then scraped off with a doctor knife. For such procedures to be effective, the coating formulation must be in a highly viscous, pasty form. For many functionalities, it is not possible to bring the formulation into such a viscous state without adversely affecting the functionality. This may be due to the fact that thickening agents are incompatible with the functional chemical.

A further procedure sometimes employed for finishing of the textile is the use of immersion or bath techniques such as foularding. The textile is fully immersed in an aqueous solution containing the functional composition that is to be applied. Subsequent repeated cycles of drying, fixation and condensation are required to complete the operation. This leads to considerable use of resources, in particular water and energy. In general, the solutions, suspensions or dispersions used for such techniques have low concentrations of the desired functional composition

Each of the upgrading steps shown in figure 1 consists of a number of operations. Various treatments with different types of chemicals are required, depending on the nature of the substrate and desired end result.

For the upgrading steps of printing, dyeing and finishing four recurring steps can generally be distinguished which often take place in the same sequence. These treatments are referred to in the professional field as unit operations and include: impregnation (i.e. application or introduction of chemicals); reaction/fixing (i.e. binding chemicals to the substrate); washing (i.e. removing excess chemicals and auxiliary chemicals); and drying.

One drawback of the usual methods of upgrading is that per upgrading step (dyeing, coating, finishing) a number of cycles of unit operations have to be carried out to achieve the desired result. Three or more cycles of unit operations are often necessary for coating, which entails a relatively high environmental impact, a long throughput time and relatively high production costs. Four or more cycles of unit operations are even required for dyeing. The traditional dyeing process requires, for instance, the final operations of several rinses (washing and soaping) for rinsing out excess chemicals, such as thickening agent. Rinsing results in much use of water. Following on from the rinses is a drying process, usually consisting of a mechanical drying step using press-out rollers and/or vacuum systems followed by a thermal drying step, for instance using tenter-frames.

It is moreover usual at this moment to carry out the different upgrading steps of the textile in separate devices. This means that for instance the dyeing is performed in a number of dye baths specially suitable for the purpose, the printing and coating are carried out in separate printing devices and coating machines, while finishing is carried out by yet another device. Because the different operations are carried out individually in separate devices, the treating of the textile requires a relatively large area, usually spread over different room areas.

It has been suggested in a number of publications that a textile article may be printed using ink-jet printing technology to produce a graphic image. Ink formulations from the graphic (paper) printing sectors have generally been used for this purpose, as such formulations are already adapted for jet deposition. In particular, pigment particulate sizes and the relatively low solids contents make such inks most suitable for inkjet devices. Such formulations are not however entirely suitable for application to all textiles, in particular those where considerable absorbency is encountered. In the past, textile articles have been pretreated with a coating onto which ink droplets may be applied using standard graphic printing techniques. A process is known from United States patent No. US 4,702,742 in which a conventional printing device is used to print onto white cloth sheets. A further process is suggested in German patent application No. DE 199 30 866 in which both ink and a fixing solution are applied to a textile using a conventional inkjet head. Known methods are however only concerned with producing a graphic image and the formulations used are unsuitable as coatings for finishing.

It has also been suggested in unpublished PCT application Nos PCT/EP2004/ 010732 and PCT/EP2004/010731 both filed on 22nd September 2004, to use inkjet type nozzles for the purpose of upgrading textile substrates. The proposed method makes use of a device comprising a number of nozzles for applying one or more substances to the textile, in addition to a conveyor for transporting the textile along the nozzles. The nozzles are ordered in a number of successively placed rows extending transversely of the transporting direction of the textile article. The textile article is guided along a first row of nozzles where it may receive a first functional layer. It may then be subsequently guided along second or third rows of nozzles for receiving further functional layers. Such a process may be referred to as digital droplet deposition.

The previously proposed method provides the option of applying chemical substances in concentrated form and with an exact dosage. The desired upgrading result can thereby be achieved in only a single cycle of unit operations. By applying the chemical substances in only one process run using a number of rows of nozzles placed in series, the efficiency per process run is increased considerably. Very uniform layers can also be applied due to the precision of dosage and nozzle control that is possible. The relatively high concentration with which the chemical substances may be applied furthermore makes interim drying almost unnecessary in many cases. The nozzles of the proposed device are preferably static with the textile being guided along the nozzles. This enables relatively high processing speeds and very precise forming of patterns. A further advantage of digital droplet deposition, is that it provides the possibility of on-demand delivery. In view of the small volumes of the reservoirs associated with the nozzles, a product change can also be realized within a very short time (less than two minutes). Subsequent sections of the same textile roll may thus be subjected to different finishing procedures almost at random. Smaller series of different textile articles can thus be processed on a single upgrading device without complicated change-over operations which can also have adverse environmental and productivity impact.

It has also been suggested in unexamined patent application No. JP61-152874 to Toray Industries, to impregnate a textile sheet with a functional composition in the form of dots. Various functional compositions are suggested including antibiotics, moisture absorbents, water repellents, antistatic agents, ultraviolet rays absorbents, infrared rays absorbents, optical whitening agents, swelling agents, solvents, saponifier, embrittlement agent, inorganic granules, metal granules, magnetic material, flame retardants, resistance, oxidants, reducing agents, perfumes, etc. The document indicates that traditional photogravure roll and screen print methods produce patterns of dots that may be too large, while in spraying techniques, the dot size and quantity of product deposited is difficult to control. The document proposes impregnating a textile with a functional composition in the form of dots, wherein a mean dot diameter is 30 to 500microns and the occupied area ratio thereof is 3 to 95%. Although the document suggests the use of inkjet printing techniques, it identifies conventional inkjet devices as being unsuitable, in particular due to the high viscosity of traditional coating compositions. The document is concerned primarily with maintaining an identifiable droplet structure and preventing the droplets from running together. Furthermore, the document provides examples regarding the use of solutions but fails to address the problems of inkjet deposition of dispersions or suspensions.

Inkjet printers of various types are generally known for providing graphic images. Such printers may be desktop inkjet printers such as used in the office or home and are generally used for printing onto a particular type of paper substrate (printer paper), using small droplets (<20 pL) of water based inks containing colorants. Larger, industrial inkjet printers also exist for printing graphic images or date/batch codes onto products; these printers are typically printing onto non-porous substrates using solvent based inks containing colorants pigments. Such formulations are not however suitable for application to most textiles in particular due to lack of colour fastness. In order to print onto textiles using inkjet techniques, textile articles have in the past been pretreated with a coating onto which ink droplets may be applied. For upgrading purposes, most currently used coatings and finishing compositions are unsuitable for deposition using inkjet techniques. Industrial inkjet printers and nozzles that produce large droplets are generally designed for use with solvent based, coloured inks. Furthermore, the droplet volumes that can be jetted are extremely low, in the order of 50 pL and mostly insufficient for textile finishing, where a significant penetration into the fabric is necessary. Typical finishing formulations are mostly water based and generally have particle sizes that can cause clogging of the nozzles. Additional problems with foaming, spattering and encrustation have been encountered. While indicating that conventional inkjet devices are unsuitable for applying finishing compositions, JP61-152874 fails to provide teaching regarding how this could be improved.

The technique described in detail in the above PCT applications makes use of the continuous inkjet (henceforth CIJ) technique. According to this technique, droplets are continuously formed in the inkjet nozzles and are charged on ejection. By using an electric field droplets may either be directed to the substrate or into a gutter for recycling. Use of CIJ makes it possible to generate 64,000 to 125,000 droplets per second per droplet jet. This large number of droplets and a number of mutually adjacent heads over the whole width of the textile results in relatively high productivity and quality of the printed result. In view of the high deposition speed, a production speed of the textile substrate of about 20 metres per minute can be realized. Although CIJ is most suitable in many cases, the cost per nozzle is generally very high. Furthermore, the specifications of the fluids to be jetted are sometimes very restrictive. They must be highly shear stable and must usually be provided with conductivity agents such as corrosive salts to enable them to carry the electrical charge. There is thus a desire to use other less complex and costly nozzles of the drop-on-demand (DoD) type.

Drop-on-demand inkjets devices are generally well known from the desktop printing field. Such devices are in principle relatively cheap although high prices may be charged for commercial cartridges! Two main principles of droplet formation are common: piezoelectric actuation, whereby a droplet is formed by resonating the fluid using a piezo-actuator; and thermal actuation (bubblejet), where a droplet is ejected by local boiling of the fluid. Other methods of droplet formation are known that may be considered to fall into the category of DoD, such as valvejet devices in which miniature valves allow controlled passage of minute volumes of fluid. The principle of operation is in all cases that the droplet is formed in response to a signal. This is thus distinguished from the continuous CIJ devices in which droplets are continuously produced. Ink formulations based on pigment concentrate that may be jetted by drop on demand inkjet devices are described in US5310778 and in US6328393.

Despite the advantages of the above proposed digital finishing procedures it has been found that most currently used coatings and upgrading compositions are unsuitable for deposition using inkjet techniques. Standard industrial inkjet nozzles are generally adapted for use with solvent-based reactive inks. Furthermore, the droplet volumes that can be jetted are extremely low, in the order of 50 pL and mostly insufficient for textile coating, where a significant penetration into the fabric is necessary. Typical coating formulations are mostly water based and generally have larger particle sizes that can cause clogging of the nozzles. Additional problems with foaming, spattering and encrustation have been encountered. When working with large numbers of nozzles operating at up to 30 KHz, reliability and fault free operation are of prime importance.

### BRIEF SUMMARY OF THE INVENTION

According to the present invention, there is proposed a finishing composition for deposition by drop-on-demand inkjet technique onto a textile substrate according to the features of claim 1. By ensuring sufficient fineness of the particles, effective and reliable droplet deposition may proceed without clogging. In the present context, the term particle is intended to cover solid particles as present in dispersion and also liquid or gel like phases, present e.g. in emulsions. It is noted that 2 microns is an approximate limit for particle size. Preferably, the maximum particle size will be less than 1 micron and for thermal inkjet may even need to be less than 0.5 microns. This value will also decrease as the percentage of solids in the composition increases above 10% but will rise as the nozzle diameter increases above 50 microns. It has been found most significant that the composition is of a consistent quality in this respect. Reference to particle size smaller than a given diameter is thus intended to refer to the D₉₉ diameter or better. The composition should also not be subject to flocculation or sedimentation. This is intended to mean that the composition does not form particles greater than the given values during prolonged use or when the inkjet device is idle during its normal use. It is understood that many compositions may e.g. form sediment during prolonged storage but that this may be overcome by appropriate mixing arrangements.

In the context of the present invention, the term "finishing" is understood to mean processes that use auxiliary chemicals to change the functionality of a textile substrate rather than merely providing it with a coloured design or changing its visual appearance as is the case with conventional inkjet printing use inks and dyes. These finishing techniques are meant to improve the properties of and/or add properties to the final product. In this context it is understood to encompass both coating and impregnating and also to include other physical treatments that upgrade the functionality of the substrate. A distinction will henceforth be made between colouring and finishing. Where necessary, finishing may be understood to exclude treatments involving the deposition of particles that are applied to the substrate only because of their absorption properties between 400 and 700 nm.

The term "finishing composition" herein encompasses aqueous solutions, aqueous dispersions, organic solutions, organic dispersions, curable liquid mixtures and molten compounds that comprise an active component. According to an important advantage of the invention, the composition may be non-reactive with the substrate. In this manner, the composition may be applied to a greater diversity of substrates than would otherwise be the case.

Furthermore, the term "textile" is intended to encompass all forms of textile article, including woven textiles, knitted textiles and non-woven textiles. The term is intended to exclude fibrous articles having two-dimensional rigidity such as carpets, paper and cardboard. These fibrous articles, although sometimes referred to as textiles, are internally linked in such a way that they maintain a substantially fixed two-dimensional form. Even though they may be flexible in a third dimension they are not generally free to stretch or distort within the plane of the fibre layer, as is inherent in a true textile. Preferably the textile substrate is more than 100 meters in length and may be provided on a roll having a width of greater than 1 meter. Preferred textiles comprise cotton and/or other treated cellulosic fibres and also polyesters, polyamides, polyacrylnitril and acetates and triacetates or blends thereof.

According to a preferred embodiment for use with most common finishing agents, the vehicle is distilled, de-mineralized and/or de-ionized water.

According to the present invention there may also be provided a co-solvent. Suitable co-solvents include 2-pyrrolidone and isopropyl alcohol (IPA) present at from 0 to 5 wt%.. The co-solvent can be used to improve the solubility of the finishing agent and/or its compatibility with other agents. Incompatibility between materials is a common formulation issue.

According to an important aspect of the present invention, considerably greater quantities of residual solids may be deposited according to the present composition. The finishing composition comprises a total of residual solids in the jetted composition of more than 10 wt% and most preferably more than 15 wt%. This leads to considerably less energy use in drying and allows greater operational speed. Particularly in the case of piezo actuation, up to 20% residual solids may be jetted.

According to a yet further feature of the invention, the humectant is present at from 10 to 35 wt% in the jetted composition. The humectant may usually be in the form of a low volatility, high boiling point liquid that helps prevent crusting of the nozzle when the jets are not active. Suitable humectants for water based systems include polyhydric alcohols, glycols, polyethylene glycol, polypropylene glycol, glycerol and n-methyl pyrrolidone (NMP). Although with certain formulations it may appear that more than 5% humectant is being used, it is in fact the case that the same material may also be present as a viscosity modifier.

The finishing composition may also comprise a viscosity control agent, preferably present at from 2 to 15 wt% in the jetted composition. The viscosity control agent is an important ingredient for increasing reliability and quality as it controls the droplet formation and break up process. This material may also act as an active functional finishing component and provide some of the end user properties. Generally, high molecular weight polymers in solution should be avoided as their elasticity makes achieving jet break up difficult.. Preferably a viscosity of 2 - 15 centipoise is desired for piezo-actuation while for thermal-actuation the viscosity may be 1 - 4 centipoise, as measured at the normal operating temperature of the nozzle.

The finishing composition may further also comprise a wetting agent, preferably present at from 0.01 to 0.3 wt% in the jetted composition. The wetting agent may reduce foaming and may also lower surface tension and improve wetting of the nozzle and textile. Exemplary wetting agents include Surfynol 104E^{™}, Dynol 604 ^{™} available from Air Products. Preferably, the surface tension of the composition is between 28 and 50 dynes/cm. If the surface tension is too high, the composition will not wet the internals of the print head properly and will leave air pockets, which will prevent reliable deposition. If the surface tension of the fluid is too low, the meniscus will not form properly in the print head nozzle and fluid will spontaneously flow onto the print head faceplate (known as faceplate wetting), which will also prevent reliable jetting.

Moreover, the finishing composition may also comprise a biocide, preferably present at up to 0.5 wt% in the jetted composition. Biocide may be used to prevent bacteria growing in the composition - this may not be required if other components of the composition are sufficiently concentrated to kill bacteria. Exemplary biocides include 1,2-benzisothiazolin-3-one and Proxel GXL ^{™} available from Zeneca Specialties.

For use in solvent based systems a degassing agents may be included at up to 0.3 wt% in the jetted composition. This can serve to either scavenge or release dissolved gas from the fluid vehicle. Dissolved gas limits the maximum reliable firing frequency by creating air bubbles in the print head during operation. Suitable degassing agents include cyclohexanone oxime and Surfynol DF75 ^{™} from Air Products.

The finishing composition may further comprise a pH modifier, preferably present at up to 1 wt % in the jetted composition. The pH modifier may be used to maintain a pH at which the solids of the composition are stably dispersed, typically this is pH>7, so most modifiers are alkaline. The pH modifier may also be used to affect the chemistry of the interaction between the composition/active agent and the textile itself. Ammonia, morpholine, diethanolamine, triethanolamine and acetic acid are suitable pH modifiers. Generally, it is desirable from an inkjet perspective to use relatively neutral solutions to reduce corrosion in the print heads. Where the chemistry dictates the need for e.g. highly alkaline solutions, ceramic (piezo) print heads may be used.

The finishing composition may also further comprise a corrosion inhibitor, preferably present at up to 0.2 wt% in the jetted composition. The corrosion inhibitor may be used to prevent unwanted ions present in the fluid (usually as impurities coming from the active components) from causing corrosion of the printer.

According to a still further aspect of the present invention, the finishing agent may be chosen for its ability to withstand shear without degradation. In particular it should be stable to shear up to at least 10⁵/s. Inkjet deposition is a high shear technique and so material that is not stable to high shear may decompose and block the print head nozzle and may also cease to provide the desired application or end user properties on the substrate. While the present invention is directed to finishing compositions for DoD, it is nevertheless considered that the composition would also be suitable for other jet deposition techniques where similar conditions of pressure, shear and nozzle diameter are encountered such as valve-jet type devices.

The finishing agent may be any appropriate agent that can endow a functional property to a textile substrate, selected from the group consisting of anti-static, anti-microbial, anti-viral, anti-fungal, medicinal, anti-pilling, non-crease, flame-retardant, water-repellant, UV-protective, deodorant, wear-resistant, slip-resistant, slip enhancing, grip enhancing, stain-resistant, oil resistant, adhesive, stiffening, softening, elasticity-enhancing, pigment-binding, conducting, semi-conducting, photo-sensitive, photo-voltaic and light-emitting agents.

For use with drugs or medicinal or biologically active agents a carrier may be used and the agent may be jetted at low temperatures e.g. below 40°C. Appropriate carriers include cyclodextrines, fullerenes, aza-crown ethers and also polylactic acid (PLA). These carriers are ideally suited for attachment both to the textile fibres and to the agent. A review of these carriers is to be found in an article by Breteler et al. in Autex Research Journal, Vol. 2 No 4 entitled Textile Slow Release Systems with Medical Application, the contents of which are hereby incorporated by reference in their entirety. Alternate carriers, particularly for use with nano-particles, may be sol gel systems.

The invention also relates to a method of finishing a textile according to claim 12.

According to a feature of the method, the droplets may be dispensed from the nozzles at velocities between 5 and 15 m/s. The droplets may also be formed at frequencies of up to 30 KHz.

Preferably the nozzles are of the piezo-electric type. Such nozzles are considerably cheaper than CIJ nozzles and are less sensitive to the physical characteristics of the composition used. In particular, since greater viscosity and percentages of solids can be used, higher concentrations of active components may be jetted. Furthermore, for sensitive agents, less shear is encountered and by using ceramic heads, otherwise corrosive products may be handled.

Alternatively, thermal print heads may be employed in cases where exposure to high temperature is not at issue or is otherwise desirable. It is also considered that valve-jet devices in which microscopic valves are periodically opened and closed could provide similar functionality when used with similar compositions as defined herein.

Also preferable is that more than 30 g/m² of wet composition is deposited on the substrate, more preferably around 50 g/m².

The invention further relates to a textile article provided with a finish comprising the finishing composition as defined above.

### BRIEF DESCRIPTION OF THE DRAWINGS

Further advantages, features and details of the present invention will be elucidated on the basis of the following description of a preferred embodiment thereof.

Reference is made in the description to the annexed figures, in which:
Figure 1 shows a schematic block diagram of a conventional process for upgrading a substrate;
Figure 2 shows a view in perspective of a textile upgrader that may be employed in an embodiment of the invention;
Figure 3 is a schematic side view of the textile upgrader of figure 2;
Figure 4 is a schematic front view of the textile upgrader of figure 2;
Figure 5 is a cut-away schematic view of the textile upgrader of figure 2;
Figure 6 is a schematic representation of a preferred sequence for performing the different treatment steps for upgrading;
Figure 7 is a schematic representation of an alternative preferred sequence for performing the upgrading steps;
Figure 8 is a schematic representation of a further preferred sequence for performing the upgrading steps;
Figure 9 shows a schematic view of a portion of woven textile coated according to the invention;
Figure 10 is a cross section through the textile of Figure 9 along the line 10-10; and
Figure 11 shows a similar view to Figure 10 through a coated textile in which smaller droplets have been used.

### DESCRIPTION OF ILLUSTRATIVE EMBODIMENTS

The following is a description of certain embodiments of the invention, given by way of example only and with reference to the drawings. Referring Figures 2-5 show a textile upgrader 1 for performing the invention. The upgrader 1 is substantially as suggested in unpublished PCT application Nos PCT/EP2004/010732 and PCT/BP2004/010731 but uses drop on demand (DoD) finishing nozzles instead of continuous inkjet (CIJ) nozzles. Textile upgrader 1 is built up of an endless conveyor belt 2 driven using electric motors (not shown). On conveyor belt 2 can be affixed a textile article T for transport in the direction of arrow P1 along a housing 3 in which the textile undergoes a number of operations. Finally, the textile may be released and discharged in the direction of arrow P2. A large number of nozzles are arranged in housing 3. The nozzles are arranged on successively placed parallel beams 14. A first row 4, a second row 5, a third row 6 and so on are thus formed. The number of rows is variable (indicated in figure 5 with a dotted line) and depends among other factors on the desired number of operations. The number of nozzles per row is also variable and depends among other things on the desired resolution of the designs to be applied to the textile. In the illustrated embodiment, the effective width of the beams is about 1 m, and the beams are provided with 8 fixedly disposed inkjet heads 12, each having about 2550 nozzles of around 35 µm. Each of the nozzles can generate a stream of droplets of ink, dye or finishing composition.

In figure 5 is indicated with dotted lines that the different heads 12 are connected (electrically or wirelessly) by means of a network 15 to a central control unit 16, which comprises for instance a micro-controller or a computer. The drive of the conveyor belt 2 is also connected to the control unit via network 15'. The control unit can now actuate the drive and the individual nozzles as required.

Also arranged per row of nozzles 4-11 is a double reservoir in which the finishing composition or dye to be applied is stored. The first row of nozzles 4 is provided with reservoirs 14a, 14b, the second row 5 is provided with reservoirs 15a, 15b, the third row 6 is provided with reservoirs 16a, 16b and so on. The appropriate substance is arranged in at least one of the two reservoirs of a row.

The different reservoirs are filled with appropriate substances and the nozzles disposed in different rows are directed such that the textile article undergoes the correct treatment. In the situation shown in figure 6, reservoir 14a of the first row 4 contains cyan-coloured ink, reservoir 15a of the second row 5 contains magenta-coloured ink, reservoir 16a of the third row 6 contains yellow-coloured ink and reservoir 17a of the fourth row 7 contains black coloured ink. The textile article is provided in rows 4-7 with patterns in a dyeing/printing treatment using CIJ nozzles of 50 microns. The reservoirs of the three subsequent rows 8-10 contain one or more finishing compositions according to the present invention, with which the treated textile can be coated in three passages using DoD thermal inkjet nozzles of 35 microns. The reservoir of the eighth row 11 contains a further finishing composition with which the printed and coated textile can be finished. In this case, the nozzles are DoD thermal inkjets having openings of 30 microns. In this embodiment the textile article T is preferably treated at the position of the fifth to the eighth row with infrared radiation coming from light sources 13 in order to influence the coating and/or the finishing.

Figure 7 shows another situation in which the textile undergoes another treatment sequence. The textile article T is first of all dyed by guiding the textile along the first row 4 and second row 5 of nozzles. These rows 4, 5 have nozzles of 70 microns and apply a relatively smooth coloured coating onto the textile. In the third to fifth rows 6-8 the dyed textile is then coated as above, whereafter the final finishing step is carried out in the sixth and seventh rows 9,10.

In the embodiment shown in figure 8, the textile article is first of all guided along the first row 4 of nozzles. The nozzles in row 4 are of about 70 microns and provide a smooth full background colour to the textile over the full width. The textile article is subsequently guided along the second row 5 and third row 6 by means of the conveyor belt, wherein patterns are printed onto the prepared surface. Good definition can be achieved in the printing steps at rows 5 and 6 using fine nozzles of between 30 and 50 microns. The textile is then guided along the fourth to sixth rows 7-9 to coat the dyed and printed textile in three passages, whereafter a final finishing treatment step is performed in the seventh and eighth rows 10,11.

It is possible to treat different successively transported textile articles or sections of the textile article in different ways, in some cases even without the transport of the textile therein having to be interrupted. It is for instance possible by means of computer control of nozzles to provide successively supplied textile articles with designs and finishes which differ in each case. It is also possible to have different substances applied to the textile through an appropriate choice of the reservoirs. The first reservoirs 14a, 15a, 16a are for instance used in each case for a first type of textile, while the second reservoirs 14b, 15b, 16b are used for another type of textile.

### EXAMPLE 1

A flame retardant composition Man 10 was prepared as given in the specification shown in Table 1.

**Table 1**

| Materials | Man 10 | Percentage By Weight (%) |
|---|---|---|
| Fire-Retardant agent | Flammentin KRE 40% solution | 50 |
| Binder | PVP K30 (25% in water) (ISP) | 20 |
| Humectant | Glycerol (Aldrich) | 29.6 |
| Surfactant | 10% Zonyl FSA (Dupont) | 0.3 |
| Biocide | Proxel GXL (ISP) | 0.1 |

The physical properties of the formulation are shown in Table 2.

**Table 2**

| Property | Man 10 |
|---|---|
| Filtration (200g) | 1.0 micron easily |
| Appearance | Pale yellow, clear. Low foam. |
| Viscosity at 25 °C, cP | 7.99 |
| Surface Tension, dynes/cm | 31.3 |
| Conductivity, mS/cm | 4.90 |

Formulation Man 10 was loaded into a Trident Ultrajet II^{™} 32/96 (faceplate has 32 channels, 3 nozzles per channel) and the formulation primed relatively easily. The jet break up and droplet formation at different drop size settings for formulation Man 10 were captured using a VisionJet Optica^{™} system, which captures images of drop formation during the jetting process. At a pulse width of 17 µs (the standard setting for this print head) two droplets formed (a main drop and satellite), whilst at a pulse width of 20 µs, one droplet formed (the satellite and main drop merge).

The above example illustrates how, in addition to reduced energy consumption, substantially less chemicals are required. With current production techniques about 150 grams of wet substances (chemicals) may be needed per square meter. In digital printing, owing to more precise dispensing and less absorption in the textile, the quantity of chemical substances to be applied can be reduced to less than 50 grams of wet substance per square meter. It is hereby possible to make a saving of about 66% in the chemicals. The saving relates not only to the primary chemicals but also to the additives, such as salts, with which the substrate is pretreated in the digital process in order to facilitate the action, fixation and/or reactivity of the primary chemicals. It is expected that a saving of 66% can also be made on these additives. Finally, waste water production and the contamination impact of the waste water can be reduced by more than 90%.

Although the above example relates to a flame retardant coating, similar process parameters may be used for most conventional textile coatings.

### EXAMPLE 2

In a second proposed exemplary coating procedure according to the present invention, an 1,800 meter long and 1.6 meter wide textile substrate of bleached and dried cotton with a weight of 100 grams per square meter of substrate is subjected to coating with a water repellent coating. The coating is performed in a single process run.

In accordance with the above, the flame retardant composition would be prepared and deposited as given in the specification shown in Table 3.

**Table 3**

| | **Example 3** | **Percentage By Weight (%)** |
|---|---|---|
| UV curable organic diluent | Dipropylene glycol diacrylate (DPGDA) | 29,70 |
| UV curable organic diluent | Propoxylated (2) neopentyl glycol diacrylate (SR9003 from Sartomer) | 54,80-56,80 |
| UV curable cross linking agent | Dipentaerythritol hexaacrylate (DPHA) | 3,00 |
| Photoinitiators | Irgacure 369:1700:819 1:1:1 (all from Ciba) | 8,50 |
| Water repellent agent | Fluoralkylacrylate | 2,00 - 4,00 |

The physical properties of the formulation are shown in Table 4.

**Table 4**

| **Flame Retardant Properties** | |
|---|---|
| Viscosity (cP) | 10 |
| PH | Not applicable |
| Surface tension (dynes/cm) | 35 |
| Particle size (um) | 0,22 |
| Solids (%) | 50% |

The formulation is jetted through DoD nozzles of 50 microns at room temperature, at a rate of 10 g/m2. The selection of these parameters allow the depth of penetration of the water repellent to be controlled such that the droplet comes to lie on the surface of the textile.

After jetting the textile article is cured by exposure to UV-light. The resultant layer has a weight of approximately 10 g/m2.

Figure 9 shows a schematic view of a portion of woven textile 100 on which four pixels 102 of a water repellent coating material have been deposited. A formulation based on Example 1 using Bayguard^{™} as the active ingredient is considered appropriate. The textile 100 comprises fibres 104 arranged in a mesh with mesh openings 106 between the fibres 104. The fibre spacing is approximately 40 microns and the pixels 102 each have a diameter of approximately 100 microns. As can be seen from Figure 9, each pixel 102 effectively covers at least four complete openings 106. Additionally, it can be seen that the pixels 102 do not form a completely closed coating in that a pore 108 is formed between adjacent pixels 102.

Figure 10 is a cross section through the textile 100 of Figure 9 along the line 10-10. It can be seen that the pixels 102 are generally located on the surface of the textile, spanning the openings 106 between adjacent fibres 104. Because of the viscous nature of the coating substance, each pixel 102 partially maintains its shape and although the pixels 102 flow together in the overlap region, the individual pixels are still discernable. It can furthermore be seen that the coating substance forming the pixel 102 partially envelopes the fibres 104 on the coated surface to form a good bond therewith. The viscosity of the coating substance is chosen to ensure the correct degree of impregnation of the material.

Figure 11 shows a similar view to Figure 10 taken through a textile 100 in which smaller droplets 110 of a coating substance have been applied. The droplets 110 are of a similar size to the mesh opening 106 and tend to pass into and even through the openings. The resultant effect is less homogenous than in the case of Figure 10. It may be used to introduce a finishing composition into the substrate rather than provide a surface finish.

While the above examples illustrate preferred embodiments of the present invention it is noted that various other arrangements may also be considered which fall within the scope of the present invention as defined by the appended claims.

## Claims

1. A finishing composition for deposition by drop-on-demand inkjet technique onto a textile substrate, the composition comprising a dispersion or emulsion of a functional finishing agent in a vehicle, wherein:
the vehicle is water, present at between 60 and 90 wt% in the jetted composition;
the finishing agent is selected from the group consisting of anti-static, anti-microbial, anti-viral, anti-fungal, medicinal, anti-pilling, non-crease, flame-retardant, water-repellant, UV-protective, deodorant, wear-resistant, slip-resistant, slip enhancing, grip enhancing, stain-resistant, oil resistant, adhesive, stiffening, softening, elasticity-enhancing, pigment-binding, conducting, semi-conducting, photo-sensitive, photo-voltaic and light-emitting agents;
the total of residual solids in the jetted composition is more than 10 wt%, more preferably more than 15 wt%;
the size of particles in the dispersion or emulsion of the finishing composition is less than 2 microns, preferably less than 1 micron, more preferably, less than 0.5 microns and not subject to flocculation or sedimentation; and
the composition further comprises a humectant, present at from 10 to 35 wt% in the jetted composition.

2. The finishing composition according to claim 1, further comprising a wetting agent, preferably present at from 0.01 to 0.3 wt% in the jetted composition.

3. The finishing composition according to any preceding claim wherein the surface tension of the composition on deposition is between 28 and 50 dynes/cm.

4. The finishing composition according to any preceding claim, wherein for piezo-actuation the composition has a viscosity of 2 - 15 centipoise and for thermal-actuation the viscosity is 1 - 4 centipoise, as measured at the normal operating temperature of the nozzle.

5. The finishing composition according to any preceding claim, further comprising a co-solvent, preferably present at up to 20 wt% in the jetted composition

6. The finishing composition according to any preceding claim, further comprising a viscosity control agent, preferably present at from 2 to 15wt% in the jetted composition.

7. The finishing composition according to any preceding claim, further comprising a biocide, preferably present at up to 0.5 wt% in the jetted composition.

8. The finishing composition according to any preceding claim, further comprising a pH modifier, preferably present at up to 1 wt% in the jetted composition.

9. The finishing composition according to any preceding claim, further comprising a corrosion inhibitor, preferably present at up to 0.2 wt% in the jetted composition.

10. The finishing composition according to any preceding claim, wherein the finishing agent is stable to shear up to at least 10⁵/s.

11. The finishing composition according to any preceding claim, wherein the finishing agent comprises nano-particles carried by a sol-gel.

12. A method of finishing a textile comprising:
providing a substantially continuous supply of a textile substrate;
providing an array of drop-on-demand inkjet nozzles;
supplying to the nozzles a finishing composition according to any of the preceding claims;
selectively dispensing the composition from the nozzles in a series of droplets to deposit a predetermined distribution of droplets onto the substrate.

13. The method according to claim 12, whereby the droplets are dispensed from the nozzles at velocities between than 5 m/s and 15 m/s.

14. The method according to claim 12 or claim 13, whereby the droplets are formed at a frequency of greater than 10 KHz, preferably greater than 20 KHz.

15. The method according to any of claims 12 to 14, wherein the nozzles are of the piezo-electric type and droplets are formed by piezo-electric excitation.

16. The method according to any of claims 12 to 14, wherein the nozzles are of the thermal inkjet type and droplets are formed by localized vaporisation.

17. The method according to any of claims 12 to 14, wherein the nozzles are of the valve-jet type and droplets are formed by periodically opening a valve.

18. The method according to any of claims 12 to 17, wherein more than 30 g/m² of wet composition is deposited on the substrate, preferably more then 50 g/m².

19. A textile article provided with a finish comprising the finishing composition according to any of claims 1 to 11.

## Patentansprüche

1. Eine Endbehandlungszusammensetzung zur Abscheidung durch Drop-on-Demand-Inkjet-Technik auf ein Textilsubstrat, wobei die Zusammensetzung eine Dispersion oder Emulsion eines funktionalen Endbehandlungsmittels in einem Trägermittel umfasst, wobei:
das Trägermittel Wasser ist, zwischen 60 und 90 Gew.-% in der ausströmenden Zusammensetzung vorhanden;
das Endbehandlungsmittel aus der Gruppe ausgewählt ist, bestehend aus antistatischen, antimikrobiellen, antiviralen, antimykotischen, medizinischen, fusselfreien, knitterfreien, flammhemmenden, wasserabweisenden, UVschützenden, deodorierenden, abriebfesten, rutschbeständigen, gleitverbessernden, haftverbessernden, schmutzabweisenden, ölbeständigen, adhäsiven, versteifenden, weichmachenden, elastizitätserhöhenden, pigmentbindenden, leitfähigen, halbleitenden, lichtempfindlichen,
photovoltaischen und lichtemittierenden Mitteln;
die Gesamtmenge von verbleibenden Feststoffen in der ausströmenden Zusammensetzung mehr als 10 Gew.-%, besonders vorzugsweise mehr als 15 Gew.-% beträgt;
die Größe der Partikel in der Dispersion oder Emulsion der Endbehandlungszusammensetzung weniger als 2 Mikrometer, vorzugsweise weniger als 1 Mikrometer, besonders vorzugsweise weniger als 0,5 Mikrometer beträgt und sie nicht der Flockung oder Sedimentation unterworfen sind; und
die Zusammensetzung ferner ein Befeuchtungsmittel, zwischen 10 und 35 Gew.-% in der ausströmenden Zusammensetzung vorhanden, umfasst.

2. Endbehandlungszusammensetzung nach Anspruch 1, die ferner ein Benetzungsmittel, vorzugsweise zwischen 0,01 und 0,3 Gew.-% in der Zusammensetzung vorhanden, umfasst.

3. Endbehandlungszusammensetzung nach einem der vorhergehenden Ansprüche, wobei die Oberflächenspannung der Zusammensetzung auf der Abscheidung zwischen 28 und 50 dyn/cm liegt.

4. Endbehandlungszusammensetzung nach einem der vorhergehenden Ansprüche, wobei die Zusammensetzung für eine Piezo-Betätigung eine Viskosität von 2 - 15 Centipoise aufweist und die Viskosität für eine thermische Betätigung 1 - 4 Centipoise beträgt, gemessen bei der normalen Betriebstemperatur der Düse.

5. Endbehandlungszusammensetzung nach einem der vorhergehenden Ansprüche, die ferner ein Co-Lösungsmittel, vorzugsweise bis zu 20 Gew.-% in der ausströmenden Zusammensetzung vorhanden, umfasst.

6. Endbehandlungszusammensetzung nach einem der vorhergehenden Ansprüche, die ferner ein Viskositätskontrollmittel, vorzugsweise zwischen 2 und 15 Gew.-% in der ausströmenden Zusammensetzung vorhanden, umfasst.

7. Endbehandlungszusammensetzung nach einem der vorhergehenden Ansprüche, die ferner ein Biozid, vorzugsweise in bis zu 0,5 Gew.-% in der ausströmenden Zusammensetzung vorhanden, umfasst.

8. Endbehandlungszusammensetzung nach einem der vorhergehenden Ansprüche, die ferner einen pH-Modifikator, vorzugsweise bis zu 1 Gew.-% in der ausströmenden Zusammensetzung vorhanden, umfasst.

9. Endbehandlungszusammensetzung nach einem der vorhergehenden Ansprüche, die ferner einen Korrosionsinhibitor, vorzugsweise bis zu 0,2 Gew.-% in der ausströmenden Zusammensetzung vorhanden, umfasst.

10. Endbehandlungszusammensetzung nach einem der vorhergehenden Ansprüche, wobei das Endbehandlungsmittel bis zu einer Scherung von 10⁵/s stabil ist.

11. Endbehandlungszusammensetzung nach einem der vorhergehenden Ansprüche, wobei das Endbehandlungsmittel Nanopartikel umfasst, die von einem Sol-Gel getragen werden.

12. Verfahren zur Endbehandlung eines Textils umfassend:
- Bereitstellen einer im Wesentlichen kontinuierlichen Zuführung eines Textilsubstrats;
- Bereitstellen einer Reihe von Drop-on-Demand-Inkjet-Düsen;
- Zuführen einer Endbehandlungszusammensetzung zu den Düsen nach einem der vorhergehenden Ansprüche;
- selektives Verteilen der Zusammensetzung aus den Düsen in einer Serie von Tröpfchen, um eine vorbestimmte Verteilung der Tröpfchen auf dem Substrat aufzutragen.

13. Verfahren nach Anspruch 12, wobei die Tröpfchen aus den Düsen bei Geschwindigkeiten zwischen 5 m/s und 15 m/s verteilt werden.

14. Verfahren nach Anspruch 12 oder Anspruch 13, wobei die Tröpfchen mit einer Frequenz von mehr als 10 kHz, vorzugsweise mehr als 20 kHz, ausgebildet werden.

15. Verfahren nach einem der Ansprüche 12 bis 14, wobei die Düsen vom piezoelektrischen Typ sind und die Tröpfchen durch piezoelektrische Anregung gebildet werden.

16. Verfahren nach einem der Ansprüche 12 bis 14, wobei die Düsen vom thermischen Tintenstrahltyp sind und die Tröpfchen durch örtliche Verdampfung gebildet werden.

17. Verfahren nach einem der Ansprüche 12 bis 14, wobei die Düsen vom Ventil-Strahl-Typ sind und die Tröpfchen durch periodisches Öffnen eines Ventils gebildet werden.

18. Verfahren nach einem der Ansprüche 12 bis 17, wobei mehr als 30 g/m² einer nassen Zusammensetzung, vorzugsweise mehr als 50 g/m², auf das Substrat aufgetragen wird.

19. Textilartikel, der mit einer Endbearbeitung, die die
Endbehandlungszusammensetzung nach einem der Ansprüche 1 bis 11 aufweist, versehen ist.

## Revendications

1. Une composition de finition pour dépôt par une technique de jet d'encre par gouttelettes à la demande sur un substrat textile, la composition comprenant une dispersion or une émulsion d'un agent de finissage fonctionnel dans un véhicule, dans laquelle composition :
- le véhicule est de l'eau, présente en une proportion comprise entre 60 et 90% en poids dans la composition pour projection.
- l'agent de finition est choisi dans le groupe consistant en des agents antistatiques, anti-microbiens, anti-viraux, antifongiques, médicinaux, anti-boulochage, ne se froissant pas, ignifuges, hydrofuges, à protection UV, déodorants, résistant à l'usure, résistant au glissement, améliorant le glissement, améliorant la préhension, résistant aux taches, résistant à l'huile, adhésifs, raidissant, adoucissant, améliorant l'élasticité, fixant les pigments, conducteurs, semi-conducteurs, photosensibles, photovoltaïques et émetteurs de lumière ;
- le total des matières solides résiduelles dans la composition pour projection est supérieure à 10% en poids et le plus préférablement supérieure à 15% en poids,
- la dimension des particules dans la dispersion ou émulsion de la composition de finition est inférieure à 2 microns, de préférence inférieure à 1 micron, plus préférablement inférieure à 0,5 microns et elles sont non sujettes à flocculation ou sédimentation; et
- la composition comprend en outre un humectant, présent en une proportion de 10 à 35% en poids dans la composition à projeter.

2. La composition de finition selon la revendication 1, comprenant en outre un agent mouillant, de préférence présent dans la composition pour projection à raison de 0,01 à 0,3% en poids.

3. La composition de finition selon l'une quelconque des revendications précédentes, dans lequel la tension superficielle de la composition au moment de déposition est comprise entre 28 et 50 dynes/cm.

4. La composition de finition selon l'une quelconque des revendications précédentes, dans lequel, pour un actionnement piézo, la composition a une viscosité de 2 à 15 centipoises et pour un actionnement thermique, la viscosité est de 1 à 4 centipoises, mesurées à la température normale de fonctionnement de la buse.

5. Composition de finition selon l'une quelconque des revendications précédentes, comprenant en outre dans la composition pour projection un co-solvant, de préférence présent jusqu'à 20% en poids dans la composition pour projection.

6. La composition de finition selon l'une quelconque des revendications précédentes, comprenant en outre un agent de contrôle de viscosité, de préférence présent à raison de 2 à 15% en poids dans la composition pour projection.

7. La composition de finition selon l'une quelconque des revendications précédentes, comprenant en outre un biocide, de préférence présent jusqu'à 0,5% en poids dans la composition pour projection.

8. La composition de finition selon l'une quelconque des revendications précédentes, comprenant en outre un modificateur de pH, de préférence présent jusqu'à 1% en poids dans la composition pour projection.

9. La composition de finition selon l'une quelconque des revendications précédentes, comprenant en outre un inhibiteur de corrosion, de préférence présent jusqu'à 0,2% en poids dans la composition pour projection.

10. La composition de finition selon l'une quelconque des revendications précédentes, dans lequel l'agent de finition est stable au cisaillement allant jusqu'à au moins 10⁵ / s.

11. La composition de finition selon l'une quelconque des revendications précédentes, dans lequel l'agent de finition comprend des nano particules portées par un sol-gel.

12. Un procédé de finition d'un textile comprenant:
- la fourniture sensiblement en continu d'un substrat textile;
- la fourniture d'un réseau de buses pour jets d'encre par gouttelettes à la demande;
- la fourniture aux buses d'une composition de finissage selon une quelconque des revendications précédentes.
- la distribution sélective de la composition par les buses sous forme de séries de gouttelettes en vue de déposer une quantité prédéterminée de gouttelettes sur le substrat.

13. Procédé selon la revendication 12, dans lequel les gouttelettes sont distribuées à partir des buses à des vitesses entre 5 m/s et 15 m/s.

14. Procédé selon la revendication 12 ou la revendication 13, dans lequel les gouttelettes sont formées à une fréquence supérieure à 10 kHz, de préférence supérieure à 20 KHz.

15. Procédé selon l'une quelconque des revendications 12 à 14, dans lequel les buses sont du type piézo-électrique et des gouttelettes sont formées par des excitation piézo-électrique.

16. Procédé selon l'une quelconque des revendications 12 à 14, dans lequel les buses sont du type à jet d'encre thermique et les gouttelettes sont formées par vaporisation localisée.

17. Procédé selon l'une quelconque des revendications 12 à 14, dans lequel les buses sont du type valve à jet et les gouttelettes sont formées par l'ouverture périodique d'une soupape.

18. Procédé selon l'une quelconque des revendications 12 à 17, dans lequel plus de 30 g/m² de la composition humide est déposée sur le substrat, de préférence plus de 50 g/m².

19. Article textile pourvu d'un apprêt comprenant la composition de finition selon l'une quelconque des revendications 1 à 11.
